

## UNITED STATES PATENT OFFICE

1,935,608

## ALUMINUM-MAGNESIUM ALLOY

Robert S. Archer, Lakewood, Ohio, assignor to  
Aluminum Company of America, Pittsburgh,  
Pa., a corporation of Pennsylvania

No Drawing. Application May 21, 1930  
Serial No. 454,509

6 Claims. (Cl. 75—1)

This invention relates to aluminum-magnesium alloys containing substantial amounts of magnesium, say 5 per cent or more, up to about 20 per cent. Such alloys have certain advantageous properties but they also possess certain disadvantages. Aluminum-magnesium alloys compounded with aluminum of high purity possess high resistance to corrosion, but unfortunately such metal is relatively costly and is therefore impracticable for some purposes, with the result that for such purposes "commercial" aluminum must be used. On the other hand, the alloys made with commercial aluminum are more subject to corrosion, so that in some cases the advantage of low cost is offset or more than offset by lack of resistance to corrosive agencies. It is therefore the chief object of my present invention to provide aluminum-magnesium alloys in which the aluminum may be no better than commercial grade as regards total impurity content but which shall nevertheless exhibit a degree of corrosion resistance comparable to that heretofore obtainable only in alloys made with the expensive high-purity metal referred to. By "aluminum of commercial grade" or "commercial aluminum" I mean such aluminum as the ordinary ingot metal of commerce, which, as is well known, averages not more than about 99.2 or 99.3 per cent pure, the remainder being for the most part silicon and iron, sometimes with small amounts of copper.

I have found that of the impurities usually present in amounts sufficient to have an important effect upon the corrosion resistance of aluminum alloys of high magnesium content, say 5 per cent or more, iron is the most detrimental; and I have determined further, by tests made with an aqueous solution containing 20 per cent of sodium chlorid and 0.3 per cent of hydrogen peroxid, that the iron impurity should be less, or in any case not greater, than the silicon impurity. I am thus able, by using aluminum of low iron impurity, though relatively high in silicon impurity, to provide aluminum-magnesium alloys possessing corrosion resistance adequate for uses in which resistance to corrosive agencies is of prime importance.

In the tests referred to above the concentration of hydrogen peroxid was maintained substantially constant and the time of immersion of the test specimens was forty-eight hours. The corrosion resistance was judged visually by examination with the naked eye and with the microscope, and quantitatively by weight of the ignited corrosion product. Taking as a standard

an alloy containing 10 per cent of magnesium, 0.04 per cent of copper, 0.10 per cent of silicon and 0.02 per cent of iron (a total of 0.12 per cent for the last two), I find that with an alloy of the same magnesium and 0.05 per cent iron content but containing 0.99 per cent of silicon the corrosion (by weight of the corrosion product) was only 13 per cent greater than in the case of the standard alloy, and with 0.10 per cent silicon and 1.01 per cent iron the corrosion was 695 per cent greater than the standard. Typical results, found with alloys containing 10 to 10.68 per cent of magnesium, are tabulated as follows, the corrosion of the standard (designated A) being taken as unity for purposes of comparison:

Table 1.—Low silicon, increasing iron

| Alloy | Percent Cu | Percent Si | Percent Fe | Percent Si+Fe | Corrosion | 75 |
|-------|------------|------------|------------|---------------|-----------|----|
| A     | 0.04       | 0.10       | 0.02       | 0.12          | 1.00      |    |
| B     | 0.05       | 0.07       | 0.26       | 0.33          | 3.35      |    |
| C     | 0.05       | 0.07       | 0.56       | 0.63          | 6.19      |    |
| D     | 0.05       | 0.10       | 1.01       | 1.11          | 7.95      |    |

Table 2.—Increasing silicon, iron 0.05%

| Alloy | Percent Cu | Percent Si | Percent Fe | Percent Si+Fe | Corrosion | 85 |
|-------|------------|------------|------------|---------------|-----------|----|
| A     | 0.04       | 0.10       | 0.02       | 0.12          | 1.00      |    |
| E     | 0.05       | 0.25       | 0.05       | 0.30          | 1.19      |    |
| F     | 0.05       | 0.57       | 0.05       | 0.62          | 1.21      |    |
| G     | 0.05       | 0.99       | 0.05       | 1.04          | 1.13      |    |

Table 3.—Increasing silicon, iron 0.60±0.05%

| Alloy | Percent Cu | Percent Si | Percent Fe | Percent Si+Fe | Corrosion | 95 |
|-------|------------|------------|------------|---------------|-----------|----|
| A     | 0.04       | 0.10       | 0.02       | 0.12          | 1.00      |    |
| C     | 0.05       | 0.07       | 0.56       | 0.63          | 6.19      |    |
| H     | 0.06       | 0.23       | 0.65       | 0.88          | 5.90      |    |
| I     | 0.06       | 0.34       | 0.64       | 0.98          | 5.28      |    |

Table 4.—Decreasing silicon, increasing iron

| Alloy | Percent Cu | Percent Si | Percent Fe | Percent Si+Fe | Corrosion | 100 |
|-------|------------|------------|------------|---------------|-----------|-----|
| A     | 0.04       | 0.10       | 0.02       | 0.12          | 1.00      | 105 |
| G     | 0.05       | 0.99       | 0.05       | 1.04          | 1.13      |     |
| F     | 0.05       | 0.57       | 0.05       | 0.62          | 1.21      |     |
| J     | 0.06       | 0.30       | 0.35       | 0.65          | 2.45      |     |
| L     | 0.06       | 0.34       | 0.64       | 0.98          | 5.28      |     |
| H     | 0.06       | 0.23       | 0.65       | 0.88          | 5.90      |     |
| D     | 0.05       | 0.10       | 1.01       | 1.11          | 7.95      |     |

Adding 0.05 per cent of copper to the 0.33 and 0.30 per cent of silicon-plus-iron of alloys B and E respectively, we have 0.38 and 0.35 per cent of copper and silicon-plus-iron, making these alloys 5 considerably better than would be considered commercial metal. Nevertheless alloy B, which contained three times as much iron as silicon, suffered more than three times as much corrosion as did the standard alloy A, the actual increase being  $3.35 - 1.00 = 2.35$  per cent of 1.00; whereas alloy E, containing only 0.03 per cent less silicon-plus-iron but having five times as much silicon as iron, showed only 19 per cent ( $1.19 - 1.00 = 0.19$  per cent of 1.00) more corrosion than 10 the standard. In alloys C and F (each containing 0.05 per cent of copper) the difference in their content of silicon-plus-iron is only 0.01 per cent; but alloy C, containing 0.56 per cent of iron and only 0.07 per cent silicon, showed a corrosion 15 six times that of the standard, an increase of 500 per cent over the latter, whereas alloy F, containing (in addition to 0.05 per cent copper) 0.05 per cent of iron and 0.57 per cent silicon, showed only 21 per cent greater corrosion than the 20 standard. Similarly in alloy D, containing 0.05 per cent copper, 0.10 per cent silicon and 1.01 per cent iron, the corrosion was nearly 600 per cent more than in the standard alloy, while in alloy G, containing 0.05 per cent copper, 0.99 per 25 cent silicon and 0.05 per cent iron, the corrosion was only 13 per cent more than the standard.

The effect of varying proportions of silicon and iron is indicated in Table 4. Alloys G and D differ in silicon-plus-iron content by only 0.07 30 per cent; and yet alloy D, in which the silicon to iron ratio is 1:10, has more than seven times the corrosion of alloy G in which the silicon to iron ratio is approximately 20:1, more than 6.5 times the corrosion of alloy F in which the ratio 35 is 11:1, and more than three times the corrosion of alloy J in which the ratio is less than 1:1. Alloys G and D, approximately 98.9 and 98.8 per cent pure, would be considered about equal in 40 grade, yet as regards corrosion resistance D is very bad while G is practically as good as the highly pure alloy A.

The effect of iron described above in commercial aluminum-magnesium alloys has been found to hold over a range of magnesium content from 50 about 5 per cent to about 16 per cent and in some cases more, the corrosion loss increasing as the iron content is increased, or, alternatively, the corrosion resistance increasing as the iron content is decreased, in respect to the silicon content. I am therefore able, using aluminum of 55 relatively low purity, as for example 99.0 pure, which is lower or at any rate no higher than the average of present commercial ingot aluminum, to provide aluminum-magnesium alloys having 60 corrosion resistance comparable to that of alloys made with aluminum of high purity, say 99.85 per cent pure. The magnesium may be of ordinary commercial grade (say 99.0 per cent pure) or better, since the amount of iron ordinarily 65 found in magnesium is very small at most; and for the further reason that the total amount of iron imported into the alloy by the magnesium

is small because the magnesium is a minor ingredient in comparison with the aluminum. In short, with commercial magnesium the amount of iron carried into the alloy by the magnesium is so slight as to be negligible.

Different lots of commercial aluminum may vary considerably not only in total impurity content but also in amount of specific impurities. For instance one lot may have more iron than will afford the degree of corrosion resistance desired for a particular purpose and may therefore be unusable, while another lot may have less iron than necessary. In such cases the first lot may often be used by mixing the two. In some cases the iron content may be brought down to 80 a usable amount by mixing more or less highly pure aluminum with the high iron metal. Or both expedients may be employed. Thus by proper selection and combination of cheaper grades of aluminum, sometimes with admixture of a relatively small amount of pure metal, it is possible to produce an alloy of adequate corrosion resistance at lower cost than would be entailed by the use of all high-purity metal.

I have also found it possible with a given iron content, to add calculated amounts of silicon so as to obtain a silicon-iron ratio desirable for favorable corrosion resistance characteristics.

I claim—

1. Corrosion - resistant aluminum - magnesium alloy consisting of aluminum and about 5 to 16 per cent of magnesium, the alloy being of commercial grade as evidenced by a silicon-plus-iron content of from about 0.3 to 1 per cent; the ratio of silicon to iron being not less than about 1:1. 105

2. Corrosion - resistant aluminum - magnesium alloy consisting of aluminum and about 5 to 16 per cent of magnesium, the alloy being of commercial grade as evidenced by a content of silicon and iron from about 0.6 to 1 per cent and the 115 iron being from about 0.05 to 0.35 per cent; the ratio of silicon to iron being not less than about 1:1.

3. Corrosion - resistant aluminum - magnesium alloy consisting of about 5 to 16 per cent of magnesium and the balance aluminum, made of commercial aluminum and magnesium, as evidenced by a content of silicon and iron in total amount from about 0.6 to 1 per cent; the ratio of silicon to iron being not less than about 1:1. 120

4. Corrosion - resistant aluminum - magnesium alloy consisting of aluminum and about 10 per cent of magnesium, containing impurity silicon-plus-iron from about 0.3 to 1 per cent; the silicon to iron ratio being not less than about 1:1. 125

5. Corrosion - resistant aluminum - magnesium alloy consisting of aluminum and about 10 per cent of magnesium, together with silicon and iron in total amount from about 0.3 to 1 per cent; the iron being not more than about 0.1 per cent. 130

6. Corrosion - resistant aluminum - magnesium alloy consisting of aluminum and about 10 per cent of magnesium, together with 0.6 to 1 per cent of silicon-plus-iron, the ratio of silicon to iron being greater than 1:1. 135

ROBERT S. ARCHER.